

1

2,784,091

**4-HYDROXY-6-ALKYL-1,3,3a,7-TETRAZAINDENE STABILIZERS FOR PHOTOGRAPHIC EMULSIONS SENSITIZED WITH POLYALKYLENE ESTERS, AMIDES, AND ETHERS**

Burt H. Carroll and Norman F. Beach, Rochester, N. Y., assignors to Eastman Kodak Company, Rochester, N. Y., a corporation of New Jersey

No Drawing. Application April 29, 1954,  
Serial No. 426,545

14 Claims. (Cl. 96—108)

This invention relates to fog inhibiting agents and stabilizers for photographic emulsions and to photographic emulsions containing them.

This application is a continuation-in-part of our application Serial No. 365,550, filed July 1, 1953, now U. S. Patent 2,716,062.

It is well known that photographic emulsions on storage tend to lose sensitivity and to become spontaneously developable without exposure to light. There is normally a detectable amount of the silver salt reduced during development in the areas where no exposure was given; this is commonly called "fog," and sometimes called "chemical fog" where it is necessary to distinguish between it and the effects of accidental exposure to radiation; in this invention, we are not concerned with the latter.

Fog depends both on the emulsion and the conditions of development; for a given emulsion it increases with the degree of development. With constant development conditions, it tends to increase with time, temperature and relative humidity of storage conditions; it is common practice to make accelerated tests of the stability of photographic emulsions by storage at increased temperature or humidity, or both. It is, of course, desirable to have emulsions as stable as possible under the conditions of high temperature and humidity which may occur in tropical climates, for example. Fog usually appears over the whole area of the sensitive coating, but when severe, it frequently is non-uniform. Fog may also be caused by exposure to chemicals, for example, hydrogen sulfide and other reactive sulfur compounds, hydrogen peroxide vapor, and strongly reducing materials. While antifoggants and stabilizers may protect, to some extent, against such effects, it is normally understood that an antifoggant protects against spontaneous growth of fog during prolonged storage or storage at high temperatures and humidities, or during development to maximum contrast and speed, or both.

It is known that the effective sensitivity of photographic silver halide emulsions may be increased by adding to them derivatives of alkylene oxides such as ethylene oxide polymers having molecular weights of 300 or more. The practical value of these compounds is severely limited by their tendency to increase fog on storage of the photographic film, especially storage at elevated temperatures and humidities. It has been found difficult to control this by the antifoggants commonly available without using quantities of antifoggant which partly neutralize the speed increase obtained from the alkylene oxide derivatives.

It is therefore an object of the present invention to provide a method for stabilizing photographic emulsions sensitized with alkylene oxide derivatives such as polyethylene oxides. A further object is to provide a means for reducing the fog produced under keeping of emulsions so sensitized, especially emulsions stored under tropical or other adverse conditions. A still further object is to provide a means for stabilizing the speed and

2

contrast of emulsions so sensitized. Other objects will appear from the following description of our invention.

These objects are accomplished in general by adding 4-hydroxy-6-alkyl-1,3,3a,7-tetraazaindene as stabilizing and fog inhibiting agents, to silver halide emulsions sensitized with condensation products of alkylene oxides with aliphatic acids, aliphatic amines or phenols. In some cases the emulsion may be sensitized with the alkylene oxide condensation products without adding the stabilizing agent.

The alkylene oxide polymers used to sensitize the emulsions may be of various types. The alkylene oxides from which the polymers are derived contain from 2 to 4 carbon atoms, e. g., ethylene oxide, propylene oxide and butylene oxide. The preparation of polymers from these compounds is described in Ellis, *The Chemistry of Synthetic Resins* (1935), pages 990 to 994. These compounds are also referred to as polyalkylene glycols and their use as sensitizers for silver halide emulsions is described in U. S. Patents 2,423,549 and 2,441,389.

The alkylene oxide condensation products include condensation products of alkylene oxides with aliphatic acids, e. g., lauric acid and glycine, condensation products of alkylene oxides with aliphatic amines or amides, e. g., glycine and lauryl amide, and condensation products of alkylene oxides with phenols, e. g., phenol itself. The preparation of these condensation products is described in U. S. Patent 1,970,578 and in Carroll U. S. application Serial No. 426,543, now Patent No. 2,743,180, filed concurrently herewith.

In each case the polyalkylene oxide or derivative of alkylene oxide should have a molecular weight of at least 300 and preferably a molecular weight of 1500 to 4000 or more.

The tetraazaindene stabilizing agents which we propose to use have the following probable structure:



in which R is an alkyl group, e. g. methyl, ethyl, propyl, butyl, etc.

The compounds of our invention may be prepared by heating ethyl acetoacetate or its homologues with 3-amino-1,2,4-triazole. (Ber. 42, Part 4, page 4642, 1909; Zeitschrift für wissenschaftliche Photographie, 47, part 1-3, page 6, 1952.) While the literature indicates that this reaction produces compounds having the general formula expressed above and the specific formula which follows, we include within the scope of our invention any isomeric or tautomeric forms of the compounds which may be produced by this reaction and which are effective fog-inhibiting or stabilizing agents for photographic emulsions.

A specific example of this class of compounds is the following:



65 4-hydroxy-6-methyl-1,3,3a,7-tetraazaindene (6-methyl-1,3-triazo-7,0'-pyrimidine-4-hydroxylic acid)

The principal purpose of our invention is to provide a means for maintaining the sensitivity and fog of silver halide emulsions at or close to initial optimum values under conditions of high temperature or humidity or both. Preferably the fog inhibitors which we propose

to use are added to the emulsion at any stage during the process of manufacture prior to coating the emulsion. The tetrazaindene fog inhibitor may be added to the emulsion in solution in any convenient solvent not injurious to the emulsion such as lower alcohols or ketones.

A solution of the tetrazaindene which we employ when added in suitable concentration before coating to unsensitized or optically sensitized silver halide emulsions usually does not appreciably affect the sensitivity and fog when measurements are made soon after coating. However, when sensitometric measurements are made after appreciable intervals of time under tropical or dry conditions of storage at elevated temperatures, these compounds do stabilize speed and maintain fog at a low level.

The preparation of silver halide emulsions involves three separate operations: (1) the emulsification and digestion or ripening of the silver halide, (2) the freeing of the emulsion from aqueous soluble salts usually by washing, (3) the second digestion or after-ripening to obtain increased sensitivity (Mees, *The Theory of the Photographic Process*, 1942, page 3). The fog inhibiting agents may be added at any stage, preferably after the final digestion.

The photographic emulsions which we use are of the developing-out type and best results have been obtained with gelatino-silver bromoiodide emulsions. However, emulsions of varying halide content may be used.

The emulsions may be chemically sensitized by any of the accepted procedures, in addition to or in combination with the sensitizing with alkylene oxide polymers. The emulsions may be digested with naturally active gelatin, or sulfur compounds may be added such as those described in Sheppard U. S. Patents 1,574,944 and 1,623,499, and Sheppard and Brigham U. S. Patent 2,410,689.

The emulsions may also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladite, which are used for sensitizing in amounts below that which produces any substantial fog inhibition, as described in Smith and Trivelli U. S. Patent 2,448,060, and as antifoggants in higher amounts, as described in Trivelli and Smith U. S. Patents 2,566,245 and 2,566,263.

The emulsions may also be chemically sensitized with gold salts as described in Waller and Dodd U. S. Patent 2,399,083, or stabilized with gold salts as described in Damschroder U. S. Patent 2,597,856 and Yutzy and Leermakers U. S. Patent 2,597,915. Suitable compounds are potassium chloroaurite, potassium aurithiocyanate, potassium chloroaurate, auric trichloride and 2-aurosulfonylbenzothiazole methochloride.

The emulsions may also be chemically sensitized with reducing agents such as stannous salts (Carroll U. S. Patent 2,487,850), polyamines such as diethylene triamine (Lowe and Jones U. S. Patent 2,518,698), polyamines such as spermine (Lowe and Allen U. S. Patent 2,521,925), or

2,728,663, Carroll and Murray U. S. Patent 2,728,664 and Leubner and Murray U. S. Patent 2,728,665.

The sensitizing and stabilizing combinations of polyalkylene oxides and tetrazaindenes are effective in the presence or absence of optical sensitizing dyes. Since optical sensitizing may affect stability of emulsions with respect to sensitivity, fog and latent image changes, the action of the compounds of this invention is not completely independent of optical sensitizing or other emulsion variables. We have found, however, that both unsensitized emulsions and emulsions sensitized with cyanine or merocyanine dyes or both may be treated with polyalkylene oxides and tetrazaindenes according to our invention.

15 The most useful concentration of the tetrazaindene compound in the emulsion is from about 0.1 gram to 4 grams per gram mole of silver halide in the emulsion. Although higher amounts may be used, no emulsion is likely to tolerate as much as 5 times this upper limit without 20 serious desensitization. Optimum concentrations are about 2.0 gram of the tetrazaindene per gram mole of silver halide. These amounts may be used in combination with one or more of the chemical sensitizing and stabilizing agents listed above.

25 The stabilizing action was determined by incubation of the emulsions usually for one or two weeks at 120° F. and constant humidity unless otherwise stated in the examples. The results of aging tests are tabulated below and compare speed, gamma and fog of the emulsions with 30 and without the stabilizing compound.

#### Example 1

One liter of a negative speed gelatino-silver bromoiodide emulsion was digested with a sulfur compound such as 35 disclosed in Sheppard U. S. Patent 1,574,944 and potassium chloroaurate and optically sensitized with 80 mg. of 3,3'-diethyl-9-methylthiacyanine bromide per mole of silver halide. To a portion of the emulsion there were added 2 grams per gram mole of silver halide of 40 the lauric acid ester of polyethylene oxide made by condensing 1 mole of lauric acid with approximately 26 moles of ethylene oxide. To a portion of this latter emulsion there was added 0.8 gram per gram mole of silver halide of 4-hydroxy-6-methyl-1,3,3a,7-tetrazaindene.

45 The emulsions were coated on film base and were exposed on an Eastman type Ib Sensitometer and developed for 6½ minutes at 68° F. in a developer of the following formula:

|    |                                |       |     |
|----|--------------------------------|-------|-----|
| 50 | N-methyl-p-aminophenol sulfate | grams | 1.5 |
|    | Hydroquinone                   | do    | 1.3 |
|    | Sodium sulfite (desiccated)    | do    | 75  |
|    | Borax                          | do    | 4.5 |
|    | Potassium bromide              | do    | 0.4 |
| 55 | Water to                       | liter | 1   |

55 The films with and without the addenda were held at 120° F. and constant humidity for one week and were then exposed and developed as in the case of the unincubated samples. The results of tests for speed, gamma and fog were as follows:

| Compound                            | Agent per mole, grams | Fresh Test |       |      | After Incubation |       |      |
|-------------------------------------|-----------------------|------------|-------|------|------------------|-------|------|
|                                     |                       | Speed      | Gamma | Fog  | Speed            | Gamma | Fog  |
| Control                             |                       | 2,700      | 0.68  | 0.10 | 1,470            | 0.58  | 0.14 |
| Polyethylene oxide lauric ester (I) | 2                     | 4,350      | .68   | .10  | 2,500            | .55   | .19  |
| I                                   |                       |            |       |      |                  |       |      |
| Tetrazaindene                       | .8                    | 4,850      | .74   | .10  | 3,800            | .63   | .13  |

bis( $\beta$ -aminoethyl) sulfide and its water-soluble salts (Lowe and Jones U. S. Patent 2,521,926).

The emulsions may also be stabilized with the mercury compounds of Allen, Byers and Murray U. S. Patent 75

#### Example 2

Coatings were made and tested as in Example 1, using instead of the lauric ester of polyethylene oxide, one gram per gram mole of silver halide of the phenol ether of poly-

ethylene oxide, made by condensing one mole of phenol with approximately 28 moles of ethylene oxide. Results of tests for speed, gamma and fog were as follows:

| Compound                             | Agent per mole, grams | Fresh Test |       |      | After Incubation |       |      |
|--------------------------------------|-----------------------|------------|-------|------|------------------|-------|------|
|                                      |                       | Speed      | Gamma | Fog  | Speed            | Gamma | Fog  |
| Control                              |                       | 2,700      | 0.68  | 0.10 | 1,470            | 0.56  | 0.14 |
| Polyethylene oxide phenol ether (II) | 1                     | 3,800      | .67   | .10  | 2,250            | .55   | .17  |
| III                                  |                       |            |       |      |                  |       |      |
| Tetrazaindene                        | .8                    | 4,350      | .67   | .10  | 3,100            | .60   | .13  |

*Example 3*

Coatings were made and tested as in Example 1, using instead of the lauric ester of polyethylene oxide, one gram per gram mole of silver halide of the condensation product of one mole of glycine with approximately 20 moles of ethylene oxide. Results of tests for speed, gamma and fog were as follows:

| Compound                        | Agent per mole, grams | Fresh Test |       |      | After Incubation |       |      |
|---------------------------------|-----------------------|------------|-------|------|------------------|-------|------|
|                                 |                       | Speed      | Gamma | Fog  | Speed            | Gamma | Fog  |
| Control                         |                       | 2,700      | 0.68  | 0.10 | 1,470            | 0.56  | 0.14 |
| Polyethylene oxideglycine (III) | 1                     | 3,500      | .67   | .10  | 2,000            | .57   | .17  |
| III                             |                       |            |       |      |                  |       |      |
| Tetrazaindene                   | .8                    | 4,050      | .72   | .09  | 2,800            | .54   | .13  |

*Example 4*

Coatings were made and tested as in Example 1, using instead of the lauric ester of polyethylene oxide, one gram per gram mole of silver halide of the condensation product of one mole of lauryl amide with approximately 20 moles of ethylene oxide. Results of tests for speed, gamma and fog were as follows:

| Compound                             | Agent per mole, grams | Fresh Test |       |      | After Incubation |       |      |
|--------------------------------------|-----------------------|------------|-------|------|------------------|-------|------|
|                                      |                       | Speed      | Gamma | Fog  | Speed            | Gamma | Fog  |
| Control                              |                       | 2,700      | 0.68  | 0.10 | 1,470            | 0.56  | 0.14 |
| Polyethylene oxide lauryl amide (IV) | 1                     | 3,800      | .70   | .10  | 1,690            | .57   | .20  |
| IV                                   |                       |            |       |      |                  |       |      |
| Tetrazaindene                        | .8                    | 4,050      | .72   | .09  | 2,800            | .54   | .13  |

The polyethylene oxide polymers used in the emulsions according to our invention may be prepared either by polymerizing ethylene oxide in the presence of aliphatic acids, aliphatic amines, or phenols, or by reacting the polymerized polyethylene oxide with aliphatic acids, acid chlorides, or esters, which produces similar products.

Instead of incorporation in the silver halide emulsion the fog-inhibitors of our invention may be incorporated in a colloid layer such as a gelatin layer in contact with the emulsion.

The fog-inhibiting agents which we have described may be used in various kinds of photographic emulsions. In addition to being useful in non-sensitized emulsions they may also be used in orthochromatic, panchromatic and X-ray emulsions. If used with sensitizing dyes, they may be added to the emulsion before or after the dyes are added. Various silver salts may be used as the sensitive salt, such as silver bromide, silver iodide, silver chloride or mixed silver halides. The azaindene compounds and alkylene oxide polymers may be used in emulsions intended for color photography, for example, emulsions containing color-forming couplers, or emulsions to be developed by solutions containing couplers.

The dispersing agents may be gelatin or other colloid such as collodion, albumen, cellulose derivatives or synthetic resins.

It will be understood that we contemplate as included within our invention all modifications and equivalents falling within the scope of the appended claims.

We claim:

1. A light-sensitive silver halide emulsion sensitized with a condensation product of 6 to 50 moles of an alkylene oxide with 1 mole of a compound selected from the

class consisting of lauric acid, lauryl amide, glycine and phenol, said alkylene oxide containing from 2 to 4 carbon atoms and said condensation product having a molecular weight of at least 300.

2. A light-sensitive silver halide emulsion sensitized with a condensation product of 6 to 50 moles of ethylene oxide with 1 mole of a compound selected from the class

30 consisting of lauric acid, lauryl amide, glycine and phenol, said condensation product having a molecular weight of at least 300.

3. A light-sensitive silver halide emulsion sensitized with an ethylene oxide polymer which is a condensation product of one mol of lauric acid with approximately 26 moles of ethylene oxide, said emulsion containing as a

50 fog-inhibiting agent 4-hydroxy-6-methyl-1,3,3a,7-tetrazaindene.

4. A light-sensitive silver halide emulsion sensitized with an ethylene oxide polymer which is a condensation product of one mol of glycine with approximately 20 moles of ethylene oxide, said emulsion containing as a fog-inhibiting agent 4-hydroxy-6-methyl-1,3,3a,7-tetrazaindene.

55 5. A light-sensitive silver halide emulsion sensitized with an ethylene oxide polymer which is a condensation product of one mol of lauryl amide with approximately 20 moles of ethylene oxide, said emulsion containing as a fog-inhibiting agent 4-hydroxy-6-methyl-1,3,3a,7-tetrazaindene.

60 6. A light-sensitive silver halide emulsion sensitized with an ethylene oxide polymer which is a condensation product of one mol of phenol with approximately 28 moles of ethylene oxide, said emulsion containing as a fog-inhibiting agent 4-hydroxy-6-methyl-1,3,3a,7-tetrazaindene.

65 7. A light-sensitive sulfur-sensitized silver halide emulsion additionally sensitized with an ethylene oxide polymer which is a condensation product of one mol of lauric acid with approximately 26 moles of ethylene oxide, said emulsion containing as a fog inhibiting agent 4-hydroxy-6-methyl-1,3,3a,7-tetrazaindene.

70 8. A light-sensitive sulfur-sensitized silver halide emulsion additionally sensitized with an ethylene oxide polymer which is a condensation product of one mol of glycine with approximately 20 moles of ethylene oxide, said emul-

75

sion containing as a fog inhibiting agent 4-hydroxy-6-methyl-1,3,3a,7-tetrazaindene.

9. A light-sensitive sulfur-sensitized silver halide emulsion additionally sensitized with an ethylene oxide polymer which is a condensation product of one mol of lauryl amide with approximately 20 moles of ethylene oxide, said emulsion containing as a fog inhibiting agent 4-hydroxy-6-methyl-1,3,3a,7-tetrazaindene.

10. A light-sensitive sulfur-sensitized silver halide emulsion additionally sensitized with an ethylene oxide polymer which is a condensation product of one mol of phenol with approximately 28 moles of ethylene oxide, said emulsion containing as a fog inhibiting agent 4-hydroxy-6-methyl-1,3,3a,7-tetrazaindene.

11. The emulsion of claim 7 which is additionally 15 chemically sensitized with gold salts.

12. The emulsion of claim 8 which is additionally chemically sensitized with gold salts.

13. The emulsion of claim 9 which is additionally chemically sensitized with gold salts.

14. The emulsion of claim 10 which is additionally chemically sensitized with gold salts.

References Cited in the file of this patent

UNITED STATES PATENTS

|           |                  |                |
|-----------|------------------|----------------|
| 1,970,578 | Schoeller et al. | Aug. 21, 1934  |
| 2,240,472 | Swan             | Apr. 29, 1941  |
| 2,400,532 | Blake et al.     | May 21, 1946   |
| 2,423,549 | Blake et al.     | July 8, 1947   |
| 2,441,389 | Blake            | May 11, 1948   |
| 2,449,225 | Heimbach et al.  | Sept. 14, 1948 |
| 2,450,397 | Heimbach         | Sept. 28, 1948 |
| 2,716,062 | Carroll et al.   | Aug. 23, 1955  |